

Jan. 12, 1965

D. PEARLMAN

3,165,457

DIRECT POSITIVE PHOTOCONDUCTOGRAPHY

Filed May 15, 1961



Fig. 1



Fig. 2



Fig. 3

DONALD PEARLMAN  
INVENTOR

BY *R. Frank Smith*  
*Emerson Holmes*  
ATTORNEYS

# United States Patent Office

3,165,457

Patented Jan. 12, 1965

1

3,165,457

**DIRECT POSITIVE PHOTOCONDUCTOGRAPHY**  
Donald Pearlman, Rochester, N.Y., assignor to Eastman  
Kodak Company, Rochester, N.Y., a corporation of  
New Jersey

Filed May 15, 1961, Ser. No. 109,977

8 Claims. (Cl. 204—18)

The present invention relates to electrolytic recording and particularly to photoconductography.

Photoconductography forms a complete image at one time or at least a non-uniform part of an image as distinguished from facsimile which at any one time produces only a uniform dot. The present invention relates to a photoconductographic process in which a positive image is produced directly.

Cross reference is made to the following series of applications filed on July 28, 1960.

Serial No. 45,940, John W. Castle Jr., "Photoconductography Employing Reducing Agents."

Serial No. 45,941, Raymond F. Reithel, "Photoconductolithography Employing Nickel Salts," now abandoned.

Serial No. 45,942, Raymond F. Reithel, "Photoconductolithography Employing Magnesium Salts," now U.S. Patent 3,053,179.

Serial No. 45,943, Raymond F. Reithel, "Photoconductography Employing Spongy Hydroxide Images," now abandoned.

Serial No. 45,944, Raymond F. Reithel, "Method for Making Transfer Prints Using a Photoconductographic Process."

Serial No. 45,945, Raymond F. Reithel, "Photoconductography Employing Manganese Compounds."

Serial No. 45,946, Raymond F. Reithel, "Photoconductography Employing Molybdenum or Ferrous Oxide," now abandoned.

Serial No. 45,947, Raymond F. Reithel, "Photoconductography Employing Cobaltous or Nickelous Hydroxide," now abandoned.

Serial No. 45,948, Donald R. Eastman, "Electrophotolithography."

Serial No. 45,949, Donald R. Eastman, "Photoconductolithography Employing Hydrophobic Images."

Serial No. 45,950, Donald R. Eastman and Raymond F. Reithel, "Photoconductography Employing Electrolytic Images to Harden or Soften Films," now U.S. Patent 3,106,516.

Serial No. 45,951, Donald R. Eastman and Raymond F. Reithel, "Photoconductography Employing Absorbed Metal Ions," now abandoned.

Serial No. 45,952, Donald R. Eastman and Raymond F. Reithel, "Photoconductography Employing Spongy Images Containing Gelatin Hardeners," now U.S. Patent 3,106,517.

Serial No. 45,953, John J. Sagura, "Photoconductography Employing Alkaline Dye Formation," now U.S. Patent 3,057,787.

Serial No. 45,954, John J. Sagura and James A. Van Allen, "Photoconductography Employing Quaternary Salts."

Serial No. 45,955, Franz Urbach and Nelson R. Nail, "Uniform Photoconductographic Recording on Flexible Sheets," now abandoned.

Serial No. 45,956, Franz Urbach and Nelson R. Nail, "High Contrast Photoconductographic Recording," now abandoned.

Serial No. 45,957, Nicholas L. Weeks, "Photoconductography Involving Transfer of Gelatin."

Serial No. 45,958, Donald R. Eastman, "Photoconductolithography Employing Rubeanates," now U.S. Patent 3,095,808.

2

Serial No. 45,959, Donald R. Eastman and Raymond F. Reithel, "Electrolytic Recording With Organic Polymers," now U.S. Patent 3,106,155.

Serial No. 46,034, Franz Urbach and Donald Pearlman, "Electrolytic Recording," now abandoned.

Cross reference is also made to the following three applications filed October 25, 1960:

Serial No. 64,901, "Simultaneous Processing in Photoconductography," Franz Urbach.

Serial No. 64,902, "Solid Recording System for Photoconductography," Nelson R. Nail.

Serial No. 64,903, "A Two-Step Reversal Processing Method in Photoconductography," Franz Urbach.

Electrolytic facsimile systems are well known. Electrolytic photoconductography is also known and is described in detail in British 188,030 Von Bronk and British 464,112 Goldmann, modifications being described in British 789,309 Berchtold and Belgium 561,403 Johnson et al.

The present invention is primarily used in photoconductographic processes because its advantages (direct positive production) are greatest there. However, the invention is also useful in facsimile or any electrical recording system.

The object of the present invention is to produce a direct positive image in a simple, efficient manner and to produce such an image that is stable and has high resolution.

According to the present invention an image in the form of variations in electrical conductivity is established in a photoconductive layer such as selenium or zinc oxide in resin. In the case of selenium the image must be developed during exposure and in the case of zinc oxide photoconductors, the image may be developed either during or immediately following exposure during the period of persistence of the image.

This image of electrical conduction is converted to a visible image by a process which involves electrolytic reduction. One characteristic of the present invention which distinguishes it from former photoconductographic processes is the fact that the electrolytic reduction is employed to render a material relatively non-reactive and non-color forming. The material which has not been so reduced is then reacted with a second reagent to form a coloring material pigment or dye. Since the coloring material is formed in the non-conductive unexposed areas of the image, the resulting print is a direct positive.

Thus the essential feature of the invention involves a color forming reaction of two or more components, one of which is reducible by electrolysis and when in its reduced state does not react with the other component or components to form the colorant. When the reducible component is relatively insoluble and becomes soluble in its reduced state, as is sometimes the case, the reduction product preferably may be removed by washing before the color forming step.

Before or after exposure to establish the conductivity image, the exposed photoconductor is, or is placed, in contact with an electrically conductive layer which contains the reducible color forming component. The layer, in some cases, is on a support separate from the photoconductor and in other cases in which the photoconductor itself is to become the final support for the print, a suitable coating containing the reducible component is applied directly to the photoconductor. While the reducible component is in contact with the exposed photoconductor, an electrical potential is applied which causes current to flow through the exposed areas of the photoconductor and the adjacent areas of the reducible layer. These are referred to as the areas of higher current density.

Thus the invention requires current to be passed through the reducible layer and during the flow of this

electric current, the reducible component is reduced at the cathode and is thus rendered incapable of later reacting with the other color forming components. In those embodiments in which the reducible layer is on a separate support, it is removed from the photoconductor at this stage of the process. Whether the reducible component is on a separate support or on the photoconductor, the next step of the process consists of treating it with the other color forming component or components. These react with the unreduced material, in the unexposed areas, to form a dye or pigment. The end result is a direct positive print.

In certain color forming processes, both components are reducible to a non-reactive state, in which case either of the components may be the one subjected to electrolytic reduction.

For clarity the component which is to be subjected to the imagewise distributed electrolytic action is referred to as the reducible component or reducible salt and the other component is referred to as the color coupler or color forming reagent.

For example the reducible salt may be a diazonium salt while the color coupler is one which reacts therewith to form an azo dye. The diazonium salt is reduced electrically to a hydrozine derivative and, as is known, the azo dyes cannot be prepared by direct reaction of such hydrazine with a color coupler. The reduction of a diazonium salt to a hydrazine is well known and a description can be found in *Technique of Organic Chemistry*, A. Weissberger, vol. 2, second edition, page 518.

As a second example, the reducible component may be any of the typical couplers used in color photography which react with oxidized developers to form an indamine, indophenol, indoaniline or azomethine dyes. Moreover, this process is an example of the systems in which either component may be the electrically treated one. That is, the reducible component may alternatively be the oxidized developer which when not reduced will react with a typical coupler to form a dye, but which in its reduced or unoxidized state is unreactive.

There are many forms of this color forming reaction which may be used. Typical couplers embrace a wide variety of chemical structures. These conveniently can be classified in three groups: (1) Open chain methylene compounds, (2) cyclic methylene compounds, and (3) methine compounds. See "The Chemistry of Dye-Forming Development" by P. W. Vittum and A. Weissberger, *Journal Photographic Science*, vol. 2, 1954, pages 81 to 96. The open chain methylene compounds are represented by the type formula  $X-\text{CH}_2-Y$  in which X and Y are the same or different electron-attracting groups which render the  $\text{CH}_2-$  groups more or less strongly acidic. The reactivity of the couplers toward oxidized developer, as well as the color of the dye formed, varies widely with the different combinations of the X- and Y- groups. There is a chart on page 85 of the Vittum and Weissberger paper showing open-chain methylene couplers  $X-\text{CH}_2-Y$ , which contains most of the known activating groups. As can be seen from this chart and from the Table I on page 86, X and Y of all the known open-chain methylene couplers are reducible groups. Reduction of either X or Y destroys the coupling ability. The commoner forms of open-chain methylene compounds are  $\alpha$ -acylacetanilides and  $\alpha$ -acylaminoacetanilides. Similarly, Table II, page 87, of the paper presents cyclic methylene couplers in which the methylene group is activated by easily reducible groups. Reduction of one of the groups destroys the coupling ability. The commoner forms of cyclic or closed methylenes are the 5-pyrazolones which are reactive in the 4-position, i.e., which have a reactive methylene group adjacent to a carbonyl group. Finally Table III on page 90 presents methine couplers. Reduction of the methine linkage also destroys the coupling ability. These include phenolic compounds containing a reactive position para to the hydroxyl group.

In color photography certain couplers are preferable for the color they produce, or for various other reasons not involved in straight recording. Hence the present invention can utilize many of the couplers which are impractical for color photography as well as those which are actually used.

The above examples all involve the formation of coloring materials, pigments or dyes by organic reactions. The present invention can also be operated using inorganic systems. For example manganate ions in the form of a coating of manganese dioxide can be reduced to the manganous ion. In the oxidized form the manganate ion will react with a leuco dye and oxidize it to a color whereas the manganous ion is incapable of such reaction. In this embodiment of the invention a layer containing manganese dioxide is subjected to electric current which reduces it to be manganous form and this layer is then placed in contact with a layer containing a leuco dye.

The orientation of the print depends on whether it is on the photoconductor itself or on a separate support. One is the mirror image of the other. In projection printing, this question of orientation of the image is taken care of by properly orienting the original positive transparency through which the exposure is made. In those embodiments in which the photoconductor is exposed by contact with a positive image, the reducible layer is preferably on a separate support since the resulting orientation of the image is then identical with that of the original positive being copied.

The invention and its advantages will be fully understood from the following examples and from the description when read in connection with the accompanying drawings in which:

FIG. 1 schematically illustrates a process according to a preferred embodiment of the invention.

FIG. 2 similarly illustrates an alternative embodiment in which the final image is formed on the photoconductor.

FIG. 3 shows the process involving development during exposure of the photoconductor rather than subsequent thereto as shown in FIG. 2.

In FIG. 1 the image of a positive transparency 10 illuminated by a lamp 11 is focused by a lens 12 on a photoconductive layer 15 of zinc oxide in suitable resin binder carried on an electrically conducting support 16 which may be highly conducting paper or which preferably includes a metal foil layer. The transparency 10 is moved to the left as indicated by the arrow 17 while the photoconductive layer 15 is moved to the right as indicated by the arrow 18 so that the image and photoconductive layer move synchronously to expose the layer part at a time.

The exposed photoconductive layer 15 is then pressed in contact with a layer 25 containing a reducible material and an ionic salt to be conducting, carried on a support 26. Contact between the two layers is assured by pressure rollers 20 and 21 which act as electrodes. The electric current is supplied by a source indicated at 22. A D.C. source is shown in this figure but since the zinc oxide, electrolyte, interface acts as a rectifier, an A.C. source could be used as well and is often more convenient. The current flowing through the exposed areas of the photoconductor and the adjacent areas of the layer 25 reduces the reducible component in its layers so that the layer 25 then contains areas with the reduced moiety and areas with unreduced material corresponding to the unexposed areas of the image. The layer 25 is then washed with water as illustrated at 27 which removes the reduced material in those cases in which the latter is soluble and the unreduced material is not soluble. This is the usual situation and removal of the reduced material leads to higher quality final prints which are stable and not subject to stain. Thus, although the washing step is not essential to the operation of the invention, it is highly desirable to include such a step in actual practice of the invention. The layer 25 is then moved in contact with

the roller 30 which applies the other reagent or reagents 31 which reagents react with the unreduced material to form the colorant. This reagent 31 does not have any effect on the reduced area even if the reduced material has not been fully removed by the wash 27. Accordingly the positive print 32 consists of a dye pigment in the area corresponding only to the unexposed area of the layer 15. Thus the print 32 is a positive of the transparency 10. Further washing of the final print 32 is sometimes useful to prevent staining. In FIG. 2 the layer 15 before or after exposure is treated as indicated by the brush 34 with a solution containing the reducible component which in this case is a diazonium salt. The exposed layer 15 with the diazonium salt on the surface thereof is passed between electrodes 35 through which an A.C. current by a source 36 is applied. Current flowing through the exposed area of the layer reduces the diazonium salt to a hydrazine producing a layer 37 which is essentially a photoconductor having both an oxidized and a reduced form of a material, namely a diazonium and a hydrazine, distributed imagewise on the surface thereof. The layer 37 is then washed with water 38 and is then treated by means of a brush 39 with a coupler which forms a dye with the unreduced diazonium thereby forming a positive print 40.

Both FIGS. 1 and 2 employ zinc oxide in resin as the photoconductor and rely on the persistence of the conducting images therein. In FIG. 3, on the other hand, a transparency 43 illuminated by a lamp 41 is focused by a lens 42 to form a complete image over the area of a photoconductive layer 45 which in this case may be either selenium or zinc oxide in resin. The photoconductive layer is carried on a transparent conductive support 46 such as glass having a thin layer of metal or metal oxide on the surface thereof adjacent to the layer 45. The layer 45 is placed in contact with an image receiving sheet 48 having a reducible salt contained in a surface layer 47. Current is passed from an A.C. or D.C. source indicated schematically at 50 between the electrode 46 and the conducting support 48. The current flowing through the layer 47 reduces the reducible salt and this reduced salt then may be washed away by water 50. The unreduced moiety remaining in the layer 47 is then treated with a suitable reactant by a brush 51 to form a positive print in the layer 47.

#### Example 1

A gelatin layer containing a solution of 50 g. water, 2.5 g. of gelatin and 0.2 g. of p-N-morpholinobenzenediazonium zinc chloride, 0.2 g. potassium chloride, 1.5 cc. glycerol and 0.3 g. formalin was coated on a paper support and dried. The surface thereof was brushed lightly with a 2-5% solution of sodium chloride to moisten the surface and render it highly conducting. The layer was then pressed in contact with a zinc oxide in resin layer coated on a metal foil paper laminate which had been exposed for 400 ft. candle seconds to a halftone positive image. 70 volt D.C. potential was applied across the electrode contacting opposite sides of the sandwich and the current was allowed to flow for 5 seconds. The diazonium-gelatin layer and its paper support were then removed from the photoconductor and the surface was brushed with a 1% solution of a coupler consisting of 3-hydroxy-β-hydroxyethyl-2-naphthamide, made alkaline by the addition of sodium hydroxide. Any compound which couples with the unreduced diazonium salt just mentioned and thereby forms a dye could have been used. The coupler combines with the unreduced diazonium salt but does not form any image in the area where the hydrazine was produced. A high resolution, good density print was obtained in this example.

#### Example 2

A gelatin layer containing a solution of 50 grams water, 2.5 g. gelatin, 0.2 g. of 2-methoxy-4-pentadecylbenzenediazonium chloride, zinc chloride double salt, 0.2 g. potas-

sium chloride, 1.5 g. glycerin, and 0.3 cc. formalin was coated to a wet thickness of approximately 0.007 inch on a sheet of baryta coated paper. The surface thereof was moistened with a solution containing 2% by weight of potassium chloride and then was pressed into contact with a layer of zinc oxide in resin coated on a metal foil-paper laminate which had been exposed for 600 ft. candle seconds to a positive image. With the zinc oxide layer as cathode, 60 volts D.C. potential was applied across the electrode contacting opposite sides of the sandwich and the current was allowed to flow for 5 seconds. The paper containing gelatin and the diazonium salt was then removed from the photoconductor. The surface was bathed in an 0.4% 50:50 alcohol-water solution of 1-hydroxy-N-octadecyl-4-sulfo-2-naphthamide (coupler) at a pH of about 8-10. The coupler combines with the unreduced diazonium salt but does not form any image in the area where the hydrazine was produced. A high resolution, good density print was obtained.

#### Example 3

A gelatin layer approximately 0.005 to 0.007 inch wet thickness was prepared from 50 g. of a 5% solution of gelatin which contained 0.2 g. 2,2'-dimethoxybenzidine-tetrazonium chloride zinc chloride double salt, 0.2 gram potassium chloride, 1.5 grams glycerin, and 0.3 cc. formalin. This layer was coated on a sheet of baryta coated paper and dried. The surface thereof was moistened with a solution containing 2% by weight of potassium chloride and it was then pressed into contact with a layer of zinc oxide in resin which had been coated on a metal foil-paper laminate and which had been exposed for 600 ft. candle seconds to a positive image. Sixty volts D.C. potential was applied across the electrode contacting opposite sides of the sandwich, the zinc oxide layer being the cathode, and current was allowed to flow for 5-10 seconds. The paper containing the gelatin and the tetrazonium salt was removed from the photoconductor, the surface was bathed in an alcoholic solution of 1-hydroxy-3',5'-dicarboxy-N-octadecyl-2-naphthaniide at a pH=8.5-9. The coupler combines with the unreduced tetrazonium salt but does not form any image in the area where the material was reduced. A high resolution, good density print was obtained in this example.

#### Example 4

This example was identical with the above Example 3 except that in place of the tetrazonium reducible salt, p-nitrosodimethylaniline was used and for the coupler in place of the material specified in Example 3, a 2% solution of α-naphthol in 50:50 water-alcohol was used and a cyan dye was obtained.

#### Example 5

A gelatin layer containing a solution of 50 grams of water, 2.5 grams gelatin, 0.2 gram potassium chloride, 1.5 grams glycerin, 0.3 cc. formalin, and 0.2 gram 1-p-sulphophenyl-3-methyl-5-pyrazolone was coated to a wet thickness of 0.005 inch on gelatin-sized paper. The surface thereof was moistened with a solution containing 2% by weight of potassium chloride and then was rolled into contact with a layer of zinc oxide in resin which was coated on a metal foil-paper laminate and then exposed for 400 ft. candle seconds to a positive image. With the zinc oxide layer as the cathode, a D.C. potential of 60 volts was applied for 5 seconds across the electrode. The paper containing the gelatin and the pyrazolone was then removed from the zinc oxide surface and moistened in a solution of p-(N-morpholino)benzenediazonium zinc chloride, zinc chloride double salt, which was at a pH of 8-10. The diazonium salt combines with the unreduced coupler but does not form any image in the areas where the coupler was reduced. A high resolution, good density, positive print was obtained in this example.

## Example 6

Fifty grams of a 5% solution of gelatin containing 0.2 g. of a 1-phenyl-3-[3'-(2",4"-diamylphenoxy)-5"- (2""-sulfonylbenzamido)benzamido]benzamido-5-pyrazolone, 0.2 gram potassium chloride, 1.5 grams glycerin, 0.3 gram N-butyacetanilide and 0.3 cc. formalin prepared in a colloid mill was coated on a gelatin-sized paper support to a wet thickness of 0.007 inch. The dry surface thereof was moistened with a solution containing 2% by weight of potassium chloride. Then this was pressed into contact with a layer of zinc oxide in resin coated on a metal foil-paper laminate which had been exposed for 600 foot candle seconds to a positive image. Sixty volts A.C. potential was applied across the electrodes contacting the opposite sides of the sandwich, and current was allowed to flow for 10 seconds. The paper containing the gelatin and the pyrazolone was removed from the photoconductor. The surface was rinsed briefly with water, then bathed with a 5% solution of 4-amino-3-methyl-N,N-diethyl-aniline, freshly oxidized by the addition of a small amount of potassium persulfate and at a pH of 9-11. The unreduced pyrazolone combines with the oxidized developer but does not form an image in the area where the pyrazolone was reduced. A good density, high quality print is obtained in this example.

## Example 7

A layer approximately 0.005 to 0.010 inch wet thickness of gelatin coated on paper from a solution of 50 grams of 5% gelatin, containing 0.2 gram acetoacetanilide, 0.2 gram sodium chloride, 1.5 grams glycerine, 0.4 cc. of formalin was allowed to dry. The surface was moistened with a solution containing 2% by weight of sodium chloride. This then was pressed into contact with a layer of zinc oxide in resin, coated on a metal foil-paper laminate which had been exposed for 400 ft. candle seconds to a positive image. Sixty volts D.C. potential was applied across the electrode contacting opposite sides of the sandwich and current was allowed to flow for 10 seconds. The zinc oxide layer was the cathode. The paper then was removed from the photoconductor and the surface was bathed in a water solution of a few percent of 4-N-ethyl-N-methylsulfamido-ethyl-3-methylaniline sulfate which had been freshly oxidized with a small amount of potassium persulfate and at a pH of 9-11. The developer combines only with the unreduced coupler and therefore forms a positive image. A high resolution, good density print was obtained in this example.

## Example 8

A layer on sized paper approximately 0.005 to 0.010 inch wet thickness, coated from a solution of 50 grams of 5% gelatin, containing 0.2 gram 1-hydroxy-2-N-[2'-methoxy-4'[x"-chlorosulfonyl-3"- (4"-tert.amylphenoxy)benzamido]phenyl]-naphthamide, 0.2 g. sodium chloride, 1.5 grams glycerin, 0.4 cc. of formalin was allowed to dry. The surface was moistened with a solution containing 2% by weight of sodium chloride. This was pressed into contact with a layer of zinc oxide in resin coated on a metal foil-laminate which had been exposed for 400 ft. candle seconds to a positive image. Sixty volts D.C. potential was applied across the electrode contacting opposite sides of the sandwich and current was allowed to flow for 10 seconds. The zinc oxide layer was the cathode. Then the paper was removed from the photoconductor and the surface was bathed in a water solution of a few percent of 4 - amino-3-methyl-N,N-diethylaniline which had been freshly oxidized with a small amount of potassium persulfate at a pH of 9-11. The developer combines only with the unreduced coupler and therefore forms a positive image. A high resolution, good density print was obtained in this example.

## Example 9

A gelatin layer approximately 0.005 to 0.010 inch wet

thickness of a solution of 50 grams of 5% gelatin, containing 0.2 gram 1-hydroxy-4-phenylazo-2-(o-chlorophenyl)naphthamide, 0.2 gram sodium chloride, 1.5 grams glycerin, 0.4 cc. of formalin and 0.3 g. N-butyacetanilide, prepared in a colloid mill was coated on sized paper and was allowed to dry. The surface was moistened with a solution containing 2% by weight of sodium chloride. This then was pressed into contact with a layer of zinc oxide in resin coated on a metal foil-paper laminate which had been exposed for 400 ft. candle seconds to a positive image. Sixty volts D.C. potential was applied across the electrode contacting opposite sides of the sandwich and current was allowed to flow for 10 seconds. The zinc oxide layer was the cathode. The paper was then removed from the photoconductor and the surface was bathed in a water solution of a few percent of 4-amino-3-methyl - N,N - diethylaniline which had been freshly oxidized with a small amount of potassium persulfate at a pH of 9-11. The developer combines only with the unreduced coupler and therefore forms a positive image. A high resolution, good density print was obtained in this example.

## Example 10

A gelatin layer approximately 0.005 to 0.010 inch wet thickness of a dispersion prepared in a colloid mill from a solution of 50 grams of 5% gelatin, containing 0.2 gram 1-hydroxy-3',5'-dicarboxy-N-octadecyl-2-naphthamide, 0.2 gram sodium chloride, 1.5 grams glycerin, 0.4 cc. of formalin and 0.3 g. N-butyacetanilide was coated on baryta sized paper and was allowed to dry. The surface was moistened with a solution containing 2% by weight of sodium chloride. This was then pressed into contact with a zinc oxide layer in resin coated on a metal foil-paper laminate which had been exposed for 400 ft. candle seconds to a positive image. Sixty volts D.C. potential was applied across the electrode contacting opposite sides of the sandwich and current was allowed to flow for 10 seconds. The zinc oxide layer was the cathode. The paper then was removed from the photoconductor and the surface was bathed in a water solution of a few percent of 4-amino-3-methyl-N,N-diethylaniline oxidized with a small amount of potassium persulfate at a pH of 9-11. The developer combines only with the unreduced coupler and therefore forms a positive image. A high resolution, good density print was obtained in this example.

## Example 11

A gelatin layer containing a solution of 50 cc. of 5% gelatin, 1.5 g. glycerol, 0.2 cc. formalin, 0.2 cc. of a wetting agent, 5 cc. of 0.3% potassium permanganate which had been added slowly to the rest of the material was filtered, then coated onto a sheet of baryta coated paper with a wet thickness of 0.005 inch. If the permanganate is added slowly, manganese dioxide is obtained in very high dispersity and therefore the suspension has a light straw yellow color. The dried layer was moistened with a solution containing 2% potassium chloride and was then rolled into contact with a zinc oxide resin layer which had been coated on a metal foil-paper laminate, and which had been exposed for 800 ft. candle seconds to a halftone image. A D.C. potential of 80 volts was applied across the electrode contacting opposite sides of the sandwich and current was allowed to flow for 10 seconds. The layer containing the manganese salt was removed from the photoconductor, briefly rinsed in water, and then bathed in a 2% solution of National Solvat Blue O leuco dye (National Aniline Company) at a pH of 4.0. A blue direct positive image was formed in the areas which correspond to the unexposed or unreduced areas of the material. The print had very high resolution and good density.

## Example 12

A 7% solution of polyvinyl alcohol which contained

1% of ferric sulfate and 1 cc. glycerol was coated onto a sized paper support to a wet thickness of about .003 inch, and allowed to dry. The layer was moistened with a solution of 2% potassium chloride and then rolled into contact with a layer of zinc oxide in resin coated on a metal foil-paper laminate which had been exposed for 400 ft. candle seconds to a positive image. Eighty volts D.C. potential was applied across the electrode contacting the opposite sides of the sandwich, the zinc oxide being the cathode, and the current was allowed to flow for 8 seconds. The paper containing the polyvinyl alcohol and ferric sulfate was removed from the photoconductor. The surface then was bathed with a 1 to 2% solution of potassium ferrocyanide and a blue positive image was formed in the unexposed or unreduced layers. The image was then rinsed and dried. A good quality print was obtained in this example.

*Example 13*

This example was identical with Example 12 above except that in place of the potassium ferrocyanide, a 2% solution of ammonium thiocyanate was used. The ultimate print consisted of a red positive image formed in the unreduced area.

The invention has been described in detail with particular reference to preferred embodiments and illustrative examples thereof, but it will be understood that variations and modifications can be effected within the spirit and scope of the invention as described hereinabove and as defined in the appended claims.

I claim:

1. In a photoconductographic process the steps comprising forming in a photoconductive layer an image pattern of variations in electrical conductivity, placing the photoconductive layer in electrical contact with a light tone layer containing a uniformly distributed, substantially colorless, material, which material will react with a reagent to form a dye of a darker tone than the initial tone of said light tone layer and which material is reducible to an non-so-reactive form by the passage of electrical current, passing current through both layers with said photoconductive layer acting as a cathode, whereupon said current is distributed in accordance with said pattern to reduce said material in areas of higher current density, and subsequently treating the light tone layer with said reagent to react with the unreduced moiety in the other areas to form said dye.

2. A photoconductographic process according to claim 1 in which said uniformly distributed material and said reagent are both substantially colorless.

3. A photoconductographic process according to claim 1 in which said uniformly distributed material is a diazonium salt which is reducible by the passage of electric current to a hydrazine and in which the reagent is a coupler which couples with the unreduced diazonium salt to form an azo dye.

4. A photoconductographic process according to claim 1 in which said reagent is an oxidized photographic developer and in which said uniformly distributed material is a photographic coupler which reacts with said oxidized developer to form a dye, the coupler being selected from the group consisting of  $\alpha$ -acylacetanilides,  $\alpha$ -acylaminoacetanilides, 5-pyrazolones reactive in the 4-position and phenols reactive in the para-position.

5. A photoconductographic process according to claim 1 in which said reagent is an oxidized photographic developer and in which said uniformly distributed material is a photographic coupler which reacts with said oxidized developer to form a dye, the coupler being selected from the group consisting of open chain methylene compounds, cyclomethylene compounds and methine compounds.

6. A photoconductographic process according to claim 1 in which said uniformly distributed material is an oxidized photographic developer which when reduced is unreactive and in which said reagent is a color coupler selected from the group consisting of open chain methylene compounds, cyclomethylene compounds and methine compounds.

7. A photoconductographic process according to claim 1 in which said uniformly distributed material is a manganese compound which by the passage of current is reducible to a manganous compound and in which said reagent is a leuco dye which reacts with the manganese compound to form a color but which does not react with a manganous compound.

8. A photoconductographic process according to claim 1 in which said uniformly distributed material is a ferric salt which by the passage of current is reducible to a ferrous salt and in which said reagent is potassium ferrocyanide.

References Cited in the file of this patent

UNITED STATES PATENTS

|           |                |       |               |
|-----------|----------------|-------|---------------|
| 863,761   | Schmid         | ----- | Aug. 20, 1907 |
| 2,038,486 | Glas           | ----- | Apr. 21, 1936 |
| 2,837,471 | Law et al.     | ----- | June 3, 1958  |
| 3,010,883 | Johnson et al. | ----- | Nov. 28, 1961 |

FOREIGN PATENTS

|    |                  |               |       |               |
|----|------------------|---------------|-------|---------------|
| 45 | 6,887<br>of 1894 | Great Britain | ----- | Nov. 3, 1894  |
|    | 215,754          | Australia     | ----- | June 23, 1958 |

OTHER REFERENCES

Weissberger: Technique of Organic Chemistry, volume 2, 2nd edition, page 518, 1949.

Vittum et al.: "The Chemistry of Dye-Forming Development," Journal of Photographic Science, volume 2, 1954, pages 81-96.

Grieg, H. G.: Proceedings of the I.R.E., "The Chemistry of High-Speed Electrolytic Facsimile Recording," October 1948, pages 1224-1234.